

# United States Patent

[19]

Minagawa

[11] 3,884,692

[45] May 20, 1975

[54] **PHOTOGRAPHIC SUPPORT**

[75] Inventor: **Nobuhiko Minagawa**, Shizuoka, Japan

[73] Assignee: **Fuji Photo Film Co., Ltd.**, Kanagawa, Japan

[22] Filed: **Mar. 13, 1973**

[21] Appl. No.: **340,790**

[30] **Foreign Application Priority Data**

Mar. 14, 1972 Japan ..... 47-25881

[52] U.S. Cl. .... **96/85; 96/87 R**

[51] Int. Cl. .... **G03c 1/86**

[58] Field of Search ..... **96/85, 87**

[56] **References Cited**

UNITED STATES PATENTS

2,647,835 8/1953 Weaver ..... 96/85

|           |         |                    |       |
|-----------|---------|--------------------|-------|
| 3,169,865 | 2/1965  | Wood .....         | 96/85 |
| 3,352,682 | 11/1967 | Harris et al. .... | 96/95 |
| 3,520,242 | 7/1970  | Kemp et al. ....   | 96/85 |
| 3,525,621 | 8/1970  | Miller .....       | 96/85 |
| 3,743,537 | 7/1973  | Honjo et al. ....  | 96/85 |
| 3,769,020 | 10/1973 | Verburg .....      | 96/85 |
| 3,793,029 | 2/1974  | Parker .....       | 96/85 |

Primary Examiner—Mary F. Kelley

Attorney, Agent, or Firm—Sughrue, Rothwell, Mion, Zinn & Macpeak

[57] **ABSTRACT**

On the back of a polyolefin laminated paper, a support for photographic light sensitive material, a coating layer composed of colloidal alumina is applied in order to prevent the paper from blistering during microwave heating.

14 Claims, 2 Drawing Figures



PATENTED MAY 20 1975

3,884,692

**FIG. 1**



**FIG. 2**

## PHOTOGRAPHIC SUPPORT

## BACKGROUND OF THE INVENTION

## 1. Field of the Invention

The present invention relates to an improved support for photographic papers.

## 2. Description of the Prior Art

It has been a recent tendency the photographic light-sensitive material art to promote development processing. As a part of this trend, water-proof photographic paper has been developed and put into use. With a water-proof photographic paper comprising a paper support coated on both sides with a hydrophobic polyolefin resin the time required for washing and drying after development processing has been greatly shortened because the support does not absorb development processing solution. Such papers have, however, required the employment of a different method of drying as compared to conventional papers.

Heretofore, the drying of photographic papers subjected to development processing has usually been conducted by bringing the emulsion-coated surface of a non-dried photographic paper into contact with a heated, smooth metallic plate to thereby evaporate from the back of the photographic paper moisture contained in both the emulsion layer and the support paper, i.e., by so-called ferrotyping drying.

However, in a water-proof photographic paper ferrotyping drying cannot necessarily be said to be the optimal drying method because the support does not have permeability to water vapor. Rather, there is a tendency to use drying methods based on hot air, infrared rays or the like. One drying method of extremely high efficiency, microwave heating, has recently been considered by the art. In microwave heating, the time required for the temperature to rise due to thermal conduction is so small as to be negligible because microwave heating causes internal heat generation in the substance heated. In addition, microwave energy is absorbed most efficiently by water molecules. Therefore, microwave heating can be said to be extremely advantageous as a method for drying photographic papers.

Where drying with microwaves is applied to a water-proof photographic paper, water contained in the emulsion layer absorbs microwave energy to generate heat which contributes to the drying of the emulsion layer, while water originally contained in a slight amount in the paper constituting the support similarly functions as a heat-producing body and promotes the drying of the emulsion layer. For these reasons, the microwave drying of water-proof photographic paper will probably be rapidly put into use in the near future.

## SUMMARY OF THE INVENTION

The inventors have discovered, however, that the microwave drying of water-proof papers has two serious defects, that is:

1. Since polyolefins used in water-proof paper are completely hydrophobic due to their structure, water remaining on the back of the support after development processing tends to assume a drop-like shape, and a prolonged period of time is needed to dry such water drops with microwaves. Thus, there often occurs the phenomenon that though the emulsion layer is completely dried with microwaves, water drops remain undried on the back of the support.

2. In microwave drying blisters are liable to occur on the polyolefin film coated on the back of water-proof photographic papers.

The inventors will not herein venture to discuss in detail the cause of such blisters, but, roughly speaking, the cause is considered to be as follows; water contained in a paper support is vaporized by the microwave heating, resulting in an increase in the pressure inside the support, which leads to the deformation of the polyolefin laminated on the back of the support, the polyolefin being in a softened state.

Water drops described in item (1) above hinder the efficiency of the heating process, which is the strongest merit of microwave heating, and the blisters described in item (2) above spoil the appearance of the photographic paper to such an extent that the commercial value of the photographic papers is completely lost. Therefore, in putting microwave drying of water-proof photographic papers into use, it is necessary to remove the above-described two defects.

As a result of extensive investigations to solve these problems, the inventors reached the present invention, i.e., the above defects are overcome with a photographic support comprising a polyolefin-laminated paper having on its back a coating layer of colloidal alumina.

## BRIEF DESCRIPTION OF THE DRAWINGS

FIG. 1 is a cross sectional view of a development processing machine for water-proof photographic paper.

FIG. 2 is a perspective view of a microwave drier.

## DETAILED DESCRIPTION OF THE INVENTION

There is no particular restriction on the kind and thickness of the paper used in the invention, but paper for photographic uses, art paper, etc. having smooth surfaces and weighing 100 g/m<sup>2</sup> to 300 g/m<sup>2</sup> is preferred.

The polyolefins used in this invention are polyethylene, polypropylene and mixtures thereof in any proportion.

The polyethylene and polypropylene used may be selected from any of those in the prior art, and their equivalents, which have been used to form polyolefin laminated papers, and the improved results of the present invention are achieved with all of such materials. Preferably the polyethylene has a melt index of about 1 to about 30 and a density of about 0.91 to about 0.97, while the polypropylene has a melt index of about 0.1 to about 20 and a density of about 0.88 to about 0.91. These ranges are not limitative, however, and are merely to serve as a guideline to one skilled in the art.

The polyolefin can be used in various thicknesses, but at thicknesses much less than 1  $\mu$  insufficient water-proofing may be achieved, while no need exists to use a thickness much greater than 100  $\mu$ .

Polyolefin-laminated papers are usually prepared by casting molten polyolefin onto a running paper base, i.e., by the so-called extrusion coating method, whereby both sides of the paper are laminated or coated with polyolefin. The surface of the polyolefin-laminated paper to which an emulsion will be applied can be a glossy surface, matted surface, silk-like surface, etc. depending upon the use thereof, whereas the back of the laminated paper is usually non-glossy.

The colloidal alumina used in the invention is fibrous alumina (hydrate) 1 m $\mu$  to 1,000 m $\mu$ , preferably 10

$m\mu$  to 100  $m\mu$ , in size. Processes for producing the same and the properties thereof are explained in detail in Japanese Pat. Nos. 20150/64, 14292/65 and 570/66.

A process for providing a coating layer of colloidal alumina on the back of a photographic support comprising a polyolefin-coated paper is specifically described below.

Colloidal alumina is diluted with water or an organic solvent miscible with water to prepare a coating solution. The concentration of colloidal alumina in the coating solution is set taking into consideration the coating amount required, the viscosity of the solution suitable for the coating method employed and the like. However, usually, the concentration of solid ingredients, i.e., alumina, is in the range of from 1 g to 50 g per 1 liter of the coating solution. In addition, it does not destroy the benefits of the present invention to add various resins, dyes, matting agents such as silica, inorganic substances, and the like to the colloidal alumina coating solution in order to improve other characteristics such as the coefficient of friction, writing property and color. For instance, the additive resins can be water or organic solvent soluble resins such as polyvinyl acetate, polyvinyl alcohol, gelatin, nitrocellulose, etc., the dyes can be any dye which is not decomposed at process conditions, the matting agents can be selected from those commonly used in the art, e.g., clay, silica, etc. and appropriate inorganic substances are water soluble compounds such as sodium chloride, sodium sulfate, potassium nitrate, etc.

The thus obtained coating solution containing colloidal alumina is applied to the back of a polyolefin-laminated paper by any usual coating method such as roll coating, bar coating, gravure coating, etc.

It is sufficient to apply the colloidal alumina in an amount of not more than 1 g per 1  $m^2$  of a support (exclusive of other components), generally in an amount greater than 0.05 g/ $m^2$ . Amounts greater than 1 g/ $m^2$  can be used, if desired, but no significant increase in improved results is obtained. The 0.05 g/ $m^2$  is a more important parameter as the upper figure is non-limiting.

Activation of the polyolefin surface prior to the coating of the colloidal alumina is not particularly required, but, where resin is contained in the coating solution or where especially strong adhesion between the coating layer and the polyolefin surface is required, it is preferred to activate the polyolefin-laminated surface by corona discharge or the like, e.g., corona discharge as described in British Pat. Specification Nos. 771,234; 715,914; 870,224; 989,377; 971,058; 1,005,631; 1,060,526; 1,019,664; 1,043,703; 1,134,211 and 1,136,902; U.S. Pat. Nos. 3,411,908; 3,53,922; 3,549,406; 3,520,242; and 3,076,720; mechanical roughening as described in British Pat. Specification No. 1,076,410; flame treatment as described in U.S. Pat. Nos. 3,072,483; 3,153,683; 3,255,034; 3,375,126; 3,431,135; 3,590,107, etc. and in British Pat. Specification No. 1,010,649; elution as described in U.S. Pat. No. 2,846,727; ozone treatment as described in U.S. Pat. No. 2,715,075; radio frequency electromagnetic treatment as described in British Pat. Specification No. 1,294,116; and chromic acid treatment as described in Japanese Pat. No. 38-22148.

The characteristics required of the thus obtained backcoating layer are: it should not be delaminated during the production or use of the photographic light-

sensitive material; it should exert no harmful influence on a photographic emulsion; it should not cause sticking or adhesion to the surface emulsion layer under high humidity conditions; and it should prevent the formation of above-described water drops and blisters. The colloidal alumina coating layer in accordance with the invention satisfies all of the above-described requirements.

Furthermore, in addition to the intended microwave drying capability, the colloidal alumina also provides the substantial merits that a pasting property (ability to adhere materials to the substrate by adhesives) and a writing property, which a noncoated support does not possess, are obtained.

The method employed in this specification to rate the microwave drying capability of water-proof papers is as follows: a water-proof paper is subjected to a development processing by an usual development processing as shown in FIG. 1, and the non-dried, processes water-proof paper is dried by means of a microwave heating apparatus shown in FIG. 2.

In FIG. 1, numeral 1 denotes a water-proof photographic paper wound as a roll and 2 denotes a development processing bath.

It is to be specifically noted that no criticality is attached to the development processing of the present invention and any developing known to the art for the emulsion involved (any photographic emulsion may, of course, be used) can be used.

In FIG. 2, numeral 3 denotes a microwave generator, 4 denotes a waveguide, and 5 denotes a water-proof photographic paper which has been subjected to development processing. In FIGS. 1 and 2, the water-proof photographic paper runs in the direction indicated by the arrow.

The microwave drying capability was rated by examining the relationship between both the oscillation power and the velocity of the microwaves traveling through the waveguide and the state of the dried surface of the water-proof photographic paper.

The microwaves can be of any type known to the art which provide a sufficient drying effect. Preferably, and this range includes commercially available microwave sources, the microwaves have a frequency of about 900 MHz to 2,500 MHz.

The present invention will now be illustrated in greater detail by several non-limiting examples of preferred embodiments of the invention.

In all examples the microwaves used were of a frequency of 900 MHz to 2,500 MHz.

In Examples 1 — 3 the polyolefins were coated by extrusion coating. In Example 4 the paper base was covered by preformed polypropylene films on both sides.

#### EXAMPLE 1

Both sides of a photographic paper weighing 180 g/ $m^2$  were laminated with polyethylene (density 0.92, melting index 2.6) at a thickness of 30  $\mu$  to prepare support A. A colloidal alumina solution having the following composition was applied to the back of support A to prepare support B.

-Continued

|          |         |
|----------|---------|
| Methanol | 2 liter |
|----------|---------|

<sup>\*</sup>(the composition of ALUMINA SOL-100 is 10 wt.% Al<sub>2</sub>O<sub>3</sub>, 2 wt.% HCl and 88 wt.% water, size is in the range 1 m $\mu$  to 1000 m $\mu$ .)

The amount of solid ingredients coated to prepare support B was 1.0 g/m<sup>2</sup>.

To each of support A and support B was applied the same emulsion for color photographic paper to thereby prepare two water-proof color photographic papers.

The thus obtained water-proof color photographic papers were exposed and subjected to development processing using a standard commercial color developer and the apparatus shown in FIG. 1 and subsequently dried by means of the microwave drier shown in FIG. 2. The relationship between the running rate of the water-proof photographic paper being dried and the state of the dried surface was examined while setting the power of the microwave generator at 1.5 KW. The results shown in Table 1 were obtained.

Table 1

| Support | State of dried surface | Running rate (m/min.) |   |   |   |
|---------|------------------------|-----------------------|---|---|---|
|         |                        | 1                     | 2 | 3 | 4 |
| A       | At the back            | ○                     | ○ | ○ | ○ |
|         | Blister                | ○                     | ○ | ○ | ○ |
| B       | At the back            | ○                     | ○ | ○ | ○ |
|         | Blister                | ○                     | ○ | ○ | ○ |

In this and the following examples, "○" in the line "At the Back" means that the back of the paper is dried, while "○" means that the back of the paper is still wet or water drops remain on the back. Also, "○" in the line "Blister" means that no blisters formed on the back of the paper, while "○" means that blisters formed on the back of the paper.

As is clear from Table 1, in the water-proof photographic paper where support A is used the drying conditions where no blisters formed on the back of the paper and complete drying is attained is narrow, whereas in the water-proof photographic paper wherein support B is used the range of drying conditions is wide, the drying velocity is large and, in addition, blisters on the back of the paper do not occur.

#### Preparation of Color Photographic Emulsion Used

0.2 g of magenta coupler, 4-(3',5'-dibutyloxy carbonylphenyl azo)-5-amino-1-naphthol, was dissolved in 2 ml of tricresylphosphate. The solution was added to a 10% by weight aqueous gelatin solution containing 2 ml of a 10 weight % aqueous sodium alkyl benzene sulfonate solution and then the mixture was subjected to homogenizing to emulsify. Six g of the resulting emulsion was mixed with 20 g of a silver chlorobromide photographic emulsion containing about 30 g of silver bromide per 1 kg of the emulsion to provide the final emulsion.

#### Development Processing Used

After exposing, the color papers were developed in the solutions having the following compositions for 10 minutes;

|                                  |      |
|----------------------------------|------|
| N-methyl-p-aminophenol ½ sulfate | 2 g  |
| Sodium sulfite anhydride         | 30 g |
| Hydroquinone                     | 8 g  |
| Sodium carbonate                 | 20 g |

-Continued

|                   |     |
|-------------------|-----|
| Potassium bromide | 4 g |
| Water             | 1 l |

5 After developing and water-washing, the paper was fixed in the following solution for 4 min.

|    |                                |       |
|----|--------------------------------|-------|
| 10 | Sodium thiosulfate (anhydride) | 350 g |
|    | Sodium sulfite (anhydride)     | 10 g  |
|    | Water                          | 1 l   |

15 After fixing and water-washing, the paper was hardened in a 4% aqueous formaldehyde solution, washed with water and treated in the following dye-bleaching bath for 15 min.

|    |                            |       |
|----|----------------------------|-------|
| 20 | Thiourea                   | 60 g  |
|    | Potassium bromide          | 30 g  |
|    | Hydrochloric acid          | 30 ml |
|    | 2-amino-3-hydroxyphenadine | 0.011 |
|    | Water                      | 1 l   |

25 The paper was washed with water and then subjected to silver-bleaching in the following solution.

|    |                            |        |
|----|----------------------------|--------|
| 30 | Crystalline copper sulfate | 100 g  |
|    | Hydrochloric acid          | 100 ml |
|    | Water                      | 1 l    |

35 The paper was then washed with water, fixed in the fixing bath, washed again and then dried.

By the above treatment, a magenta image having completely bleached halide portions was obtained.

This material was favorable for the magenta component image of a multi-colored photosensitive material.

40

#### EXAMPLE 2

Both sides of a high quality paper weighing 130 g/m<sup>2</sup> were laminated with polyethylene (density 0.96, melt index 15) at a thickness of 30  $\mu$  to prepare support C.

45 On the other hand, the back of support C was subjected to corona discharge treatment at a discharge output of 4 KW and a discharge treating velocity of 100 m/min., and subsequently coated with a solution having the following composition to prepare support D.

|    |                                                           |         |
|----|-----------------------------------------------------------|---------|
| 55 | ALUMINA SOL-100, as in Example 1                          | 2 kg    |
|    | MOVINYL DMIH*(polyvinyl acetate emulsion, made by Hoechst | 0.01 kg |
|    | Gosei K.K.)                                               |         |
|    | Water                                                     | 8 liter |

\*(39 wt.% polyvinyl acetate and 70 wt.% water)

The amount of solid ingredients coated to prepare support D was 0.3 g/m<sup>2</sup>. To each of support C and support D was applied the same emulsion for black-and-white photographic paper to produce waterproof photographic papers. The thus obtained waterproof photographic papers were subjected to development processing and dried using the same apparatus as was used in Example 1. In this example, the power of the microwave generator was set at 3.0 KW, and the relationship between the running rate of the waterproof photo-

65

graphic paper in the drier and the state of dried surface was examined. The results shown in Table 2 were obtained.

Table 2

| Support | State of dried surface | Running rate (m/min.) |   |   |   |
|---------|------------------------|-----------------------|---|---|---|
|         |                        | 1                     | 2 | 3 | 4 |
| C       | At the back            | ○                     | ○ | ○ | ○ |
|         | Blister                | ○                     | ○ | ○ | ○ |
| D       | At the back            | ○                     | ○ | ○ | ○ |
|         | Blister                | ○                     | ○ | ○ | ○ |

As is evident from Table 2, in the water-proof paper wherein support C is used there is observed either remaining water drops on the back or the formation of blisters on the back under any drying conditions, which virtually makes microwave drying impossible. In contrast, in the water-proof photographic paper wherein support D is used, the state of the dried surface is good even when the running rate of the water-proof photographic paper, i.e., drying velocity, is as large as 5 m/min. Thus, the effects of coating the alumina sol to the back of support are seen to be highly beneficial.

#### Composition of Black & White Photographic Emulsion Used

|                                                                                         |            |    |
|-----------------------------------------------------------------------------------------|------------|----|
| Silver chlorobromide containing 50 mole % of silver bromide (particle size: 0.6 micron) | 28 g       | 30 |
| Gelatin                                                                                 | 120 g      |    |
| 6 weight % aqueous saponin solution                                                     | 2.5 cc     |    |
| 5 weight % aqueous chromium alum solution                                               | 5 cc       |    |
| 6 weight % aqueous formaldehyde solution                                                | 10 cc      |    |
| Water                                                                                   | to 1000 cc |    |

#### The composition of the developer used

|                                   |            |    |
|-----------------------------------|------------|----|
| p-methylaminophenol (1/2 sulfate) | 3.0 g      | 40 |
| Sodium sulfite anhydride          | 45.0 g     |    |
| Hydroquinone                      | 12.0 g     |    |
| Sodium carbonate (1 hydrate)      | 80.0 g     |    |
| Potassium bromide                 | 2.0 g      |    |
| Water                             | to 3000 cc |    |

#### EXAMPLE 3

The surface of a high quality art paper weighing 300 g/m<sup>2</sup> was laminated with polyethylene (density 0.92 g/cm<sup>3</sup>, melt index 25) and the back thereof was laminated with a mixture of polyethylene (same as above) (0.8 part by weight) and polypropylene (0.2 part by weight) of (density 0.92 g/cm<sup>3</sup>, melt index 4), each layer of a thickness of 30  $\mu$ , to prepare support E. Separately, the back of support E was subjected to corona discharge treatment at a corona discharge treating velocity of 100 m/min. and subsequently coated with a solution having the following composition to prepare support F. The strength of the corona discharge treatment was 0.05 KW per 1 cm<sup>2</sup> width. It is expressed as electrical power per unit width since the corona discharge was carried out using a bar-form electrode disposed close to the running web.

-Continued

|                                                                          |           |
|--------------------------------------------------------------------------|-----------|
| SNOWTEX-O** (colloidal silica made by Nissan Chemicals Industries, Ltd.) | 2 kg      |
| Methanol                                                                 | 10 liters |

\*(10 wt.% Al<sub>2</sub>O<sub>3</sub>, 2 wt.% acetic acid and 88 wt.% water, size is in the range 1  $\mu$  to 1000 ( $\mu$ ))

\*\*(20 wt.% SiO<sub>2</sub> and 80 wt.% water)

The amount of colloidal alumina coated to prepare support F was 0.4 g/m<sup>2</sup>. To each of support E and support F was applied the same emulsion for color photographic paper as was used in Example 1 to produce water-proof photographic papers, which, after development processing in the apparatus of FIG. 1 using a developer as in Example 1, were dried with microwaves in the same manner as in Example 2. In this example, the power of the microwave generator was 2.0 KW.

The relationship between the drying velocity and the state of the dried surface was examined. The results obtained are shown in Table 3.

Table 3

| Support | State of dried surface | Running rate (m/min.) |   |   |   |
|---------|------------------------|-----------------------|---|---|---|
|         |                        | 1                     | 2 | 3 | 4 |
| E       | At the back            | ○                     | ○ | ● | ● |
|         | Blister                | ○                     | ○ | ○ | ○ |
| F       | At the back            | ○                     | ○ | ○ | ○ |
|         | Blister                | ○                     | ○ | ○ | ○ |

From Table 3 it is seen that the effects of coating the back of the support in accordance with the present invention are evident.

#### EXAMPLE 4

Polypropylene films 20  $\mu$  in thickness (density 0.91) were laminated on both sides of a paper for photographic use weighing 200 g/m<sup>2</sup> to prepare support G. Separately, a solution having the following composition was applied to the back of support G to prepare support H.

|                 |            |
|-----------------|------------|
| ALUMINA SOL-200 | 2 kg       |
| Methanol        | 200 liters |

The amount of colloidal alumina coated to prepare support H was 0.1 g/m<sup>2</sup>. To each of support G and support H was applied the same emulsion for color photographic paper as was used in Example 1 to produce water-proof photographic papers. The resulting photographic papers were subjected to a development processing by means of the development processing machine shown in FIG. 1 using a developer as in Example 1, and then the nondried, water-proof photographic papers were dried by passing them through a microwave drier as shown in FIG. 2. In this example, the state of the dried surface was examined by changing the power of the microwave oscillation while fixing the running rate of the paper in the microwave drier to be 1 m/min.

Table 4

| Support | State of dried surface | Power of oscillation (KW) |     |   |     |
|---------|------------------------|---------------------------|-----|---|-----|
|         |                        | 0.6                       | 0.8 | 1 | 1.5 |
| G       | At the back            | ○                         | ○   | ○ | ○   |
|         | Blister                | ○                         | ○   | ○ | ○   |
| H       | At the back            | ○                         | ○   | ○ | ○   |
|         | Blister                | ○                         | ○   | ○ | ○   |

From Table 4, it is seen that coating of alumina on the back of the support prevents the formation of blisters and, in addition, the back can be dried with microwaves of low energy.

While the invention has been described in detail and with reference to specific embodiments thereof, it will be apparent to one skilled in the art that various changes and modifications can be made therein without departing from the spirit and scope thereof.

What is claimed is:

1. A photographic light-sensitive material comprising
  - a support which comprises a polyolefin-laminated paper having on its back a coating layer composed of fibrous colloidal alumina (hydrate), and
  - b. a silver halide emulsion layer on the side of said support opposite the alumina coated side.
2. A photographic light-sensitive material as claimed in claim 1, wherein both surfaces of said paper are polyolefin coated.
3. A photographic light-sensitive material as claimed in claim 1, wherein the thickness of a polyolefin layer on said paper is from 10 to 100  $\mu$ .
4. A photographic light-sensitive material as claimed in claim 1, wherein said polyolefin is polyethylene, polypropylene or a mixture of polyethylene and polypropylene.
5. A photographic light-sensitive material as claimed in claim 1, wherein the size of the alumina is from 1 to 1,000  $\text{m}\mu$ .
6. A photographic light-sensitive material as claimed in claim 1, wherein the coating amount of alumina is

more than 0.05 g/m<sup>2</sup>.

7. A photographic light-sensitive material as claimed in claim 5, wherein the size of the alumina is from 10 to 100  $\text{m}\mu$ .

8. A photographic light-sensitive material as claimed in claim 6, wherein the coating amount of alumina is less than 1 g/m<sup>2</sup>.

9. A photographic light-sensitive material as claimed in claim 1, wherein the paper has a weight of 100 g/m<sup>2</sup> to 300 g/m<sup>2</sup>.

10. A photographic light-sensitive material as claimed in claim 1, wherein the support polyolefin is polyethylene.

11. A photographic light-sensitive material as claimed in claim 1, wherein the polyolefin is polypropylene.

12. A photographic light-sensitive material as claimed in claim 1, wherein the polyolefin is polyethylenepolypropylene mixture.

13. A photographic light-sensitive material as claimed in claim 4, wherein the polyethylene has a density of about 0.91 to about 0.97 and a melt index of about 1 to about 30 and the polypropylene has a density of about 0.88 to about 0.91 and a melt index of about 0.1 to about 20.

14. A photographic light-sensitive material as claimed in claim 4, wherein:

- a. the paper has a weight of 100 g/m<sup>2</sup> to 300 g/m<sup>2</sup> and is coated on both sides with a polyolefin layer;
- b. a polyolefin layer is 10 to 100  $\mu$  thick;
- c. the alumina has a size of 1  $\text{m}\mu$  to 1,000  $\text{m}\mu$ ;
- d. the alumina is present in a layer consisting essentially of alumina in an amount of 0.05 to 1 g/m<sup>2</sup>;
- e. the polyethylene has a density of from about 0.91 to about 0.97 and a melt index of from about 1 to about 30; and
- f. the polypropylene has a density of from about 0.88 to about 0.91 and a melt index of from about 0.1 to about 20.

\* \* \* \* \*

UNITED STATES PATENT OFFICE  
CERTIFICATE OF CORRECTION

PATENT NO. : 3,884,692  
DATED : May 20, 1975  
INVENTOR(S) : Nobuhiko MINAGAWA

It is certified that error appears in the above-identified patent and that said Letters Patent are hereby corrected as shown below:

IN THE SPECIFICATION:

Column 3, line 53 - delete "3,53,922" and insert -- 3,253,922 --

Signed and Sealed this  
*twenty-first Day of October 1975*

[SEAL]

*Attest:*

**RUTH C. MASON**  
*Attesting Officer*

**C. MARSHALL DANN**  
*Commissioner of Patents and Trademarks*